# NEW EUROPEAN PATENT SPECIFICATION

(11) **EP 0 257 364 B2**
(45) Date of publication and mention of the opposition decision: **15.10.1997**
(45) Mention of the grant of the patent: 21.10.1992
(21) Application number: 87111197.7
(22) Date of filing: 03.08.1987
(51) Int. Cl.: G03G 13/08, G03G 9/10, G03G 15/00

(54) **Developing method for electrostatic latent image**
Entwicklungsverfahren für latente elektrostatische Bilder
Procédé pour développer des images latentes électrostatiques

(30) Priority: 06.08.1986 JP 183422/86; 06.08.1986 JP 183423/86
(43) Date of publication of application: 02.03.1988
(73) Proprietor: KONICA CORPORATION, Tokyo 163 (JP)
(72) Inventor: Kaneko, Tadashi Konishiroku Photo Ind. Co., Ltd., Hachioji-shi Tokyo (JP); Okuyama, Yuki Konishiroku Photo Ind. Co., Ltd., Hachioji-shi Tokyo (JP); Arai, Mitsutaka Konishiroku Photo Ind. Co., Ltd., Hachioji-shi Tokyo (JP); Yamamoto, Yoko Konishiroku Photo Ind. Co., Ltd., Hachioji-shi Tokyo (JP); Ikeuchi, Satoru Konishiroku Photo Ind. Co., Ltd., Hachioji-shi Tokyo (JP)
(74) Representative: Türk, Gille, Hrabal, Leifert

(56) References cited:
- EP-A- 0 160 503
- EP-A- 0 161 128
- EP-A- 0 188 171
- EP-A- 0 219 233
- DE-A- 3 004 152
- DE-A- 3 511 171
- DE-A- 3 540 638
- GB-A- 2 147 714
- US-A- 4 076 857
- US-A- 4 562 136
- "Recent electrophotographic development systems and the development and practical use of the toner material" (1985), p. 220

## Description

This invention relates to a method for developing electrostatic latent images and, more particularly, to a method for developing electrostatic latent images formed on a latent image carrying member in electrophotography, electrostatic recording, electrostatic printing and the like by making use of a two-component type developer.

Nowadays, as to the methods for forming a visible image from an image information, the methods such as electrophotography, electrostatic recording and electroprinting are widely utilized, in which visible images are formed through electrostatic latent images.

There are two types of developers used for developing the above-mentioned electrostatic latent images: one is the so-called two-component type developer comprising toners and carriers in the form of mixture (EP-A-0 160 503) and the other is a single component type developer comprising magnetic toners containing magnetic substances, which is used independently without mixing with carriers. In the methods for developing electrostatic latent images by making use of the former developer, that is of the two-component type, toners are frictionally charged by mechanically stirring the toners and carriers. It is, therefore, possible to control both the static chargeability and static charge potential of the toners to a considerable degree by selecting the properties of the carriers, the conditions of stirring and so forth and, further, this developer has a wide selection of colors with which the toners are endowed. The above-mentioned methods are superior to the methods for developing electrostatic latent images by making use of the latter developer of the single component type, from the above-mentioned points.

Concerning the methods of forming fixed images through the processes of developing electrostatic latent images by making use of the two-component type developers, there have so far been proposed the techniques for mixing toners and carriers smaller in size, from the viewpoint of the improvements in the resolving power and gradation reproduction or the image quality of fixed images.

In JP-A-181 362/1984, JP-A-22 847/1984, JP-A-222 851/1984, JP-A-222 852/1984, JP-A-222 853/1984 and JP-A-223 467/1984, and its combined counterpart GB-A-2 141 643 (Japanese Patent Applications Nos. 57446/1983, 96901/1983, 96902/1983, 96903/1983, and 97973/1983), for example, there is disclosed the techniques in which an electrostatic latent image formed on a latent image carrying member is developed in a non-contact developing system, by making use of a two-component type developer comprising small-sized carriers having a diameter of not larger than 50 µm and small-sized toner having a diameter of not larger than 20 um. The above-mentioned non-contact developing system is a system in which a developer layer comprising toners and carriers, which is carried on a developer transport/carrying member, is fed into a developing area so as not to bring the developer layer into direct contact with the latent image carrying member.

However, there are the following problems:

In the case of using small-sized carriers such as mentioned above, toners and carriers may hardly be frictionally charged, because the fluidity of the carriers is liable to be lowered as they are getting smaller in size.

Resultingly, the electrostatic and physical bonding strength of the carriers to a developer transport/carrying member is weakened and, similarly, the electrostatic and physical bonding strength of the carriers to the toner is also weakened.

Further, the carriers are usually transported by magnetic force being adhered to the surface of the developer transport/carrying member, in the case of using small-sized carriers, the adhesion force of the carriers to the developer transport/carrying member is weak.

As the results of the above-mentioned problems, in the course of performing a development process, the carriers or toners will fly about in an apparatus to contaminate the inside thereof, and the toners or carriers will adhere to the non-image areas of the latent image carrying member to produce fog; and, further, the carriers will adhere to the latent image carrying member to make an image unclear.

As a countermeasure to the above-mentioned problems, if the carriers are made larger in particle size so as to prevent the carriers from flying about and so forth, there will raise the following problems; a thin developer layer may hardly be formed on the developer transport/carrying member and the developer layer is liable to be uneven in thickness and, resultingly, the undesirable phenomena such as uneven imaging and imaging failure are taken place in a fixed image ultimately obtained, so that no sharp image may finally be obtained.

Meanwhile, in the course of performing development processes many times in repetition, and in the case of forming a thin developer layer on a developer transport/carrying member, that is, for example, in the case of regulating a developer layer thickness by bringing a thin layer forming member such as a blade into elastic contact with the surface of the developer transport/carrying member, the developer is applied with a strong pressure to make the toner substances adhere to the carriers with a strong physical pressure, that is to say, the so-called "filming phenomenon" is increased, so as to lower the frictional chargeability between the toners and carriers. Resultingly, various problems will be caused as follows:

Fog will be produced by the weakly charged toners; the toners will fly about; the carriers to which toner substances adhere will adhere to an electrostatic latent image so as to lower the image quality; the carriers will adhere to the electrostatic latent image so as to lower the image quality; a satisfactorily thin layer will hardly be formed on the developer/transport carrying member; and the like problems, so that no sharp image will finally be obtained.

On the other hand, to prevent the production of fog, it may be considered to make greater a minimum gap, that is a development gap, between a latent image carrying member and a developer transport/carrying member in a developing area.

However, in the case that the gap is relatively wider, a counter electrode effect is lowered in development so as to lower the developability, that is, the adhesion property of toners to an electrostatic latent image is lowered. Resultingly, an excellent development is hardly performed.

The developability may be improved by generating a relatively greater oscillatory electric field in a development area as well as by making a development gap larger though, in the case of generating such a greater oscillatory electric field as the development gap is made wider, there is such a problem that toners will adhere increasingly to the non-image portions of a latent image carrying member to produce fog and carriers will increasingly fly about to contaminate the inside of an apparatus. Further, it is necessary to electrically insulate a developing unit satisfactorily from and the designing of the units is considerably complicated, because of the generation of the greater oscillatory electric field.

This invention is based on the circumstances mentioned above.

It is, accordingly, an object of the invention to provide a developing method in which no contamination is caused inside an apparatus by both toners and carriers flying about, no fog is produced, an excellent development can be performed with a two-component type developer comprising the toner and carriers and, resultingly, a sharp image can be formed so as to be excellent in both resolving power and gradation reproduction.

Another object of the invention is to provide a developing method capable of forming a sharp image without having any uneven imaging and imaging failure.

A further object of the invention is to provide a developing method in which a thin developer layer can stably be formed on a developer transport/carrying member even in repeating development processes many times and, resultingly, excellent images can stably be formed, extending over a long period of time.

The developing method of the invention is a developing method in which a two-component type developer layer comprising toner particles and magnetic carrier particles is formed on a developer transport member and the resulted developer layer is fed into a developing area where an oscillatory electric field is generated so as to develop an electrostatic latent image on a latent image carrying member. The particular characteristic is that the developer layer formed on the developer transport mermber has a thickness of not more than 1000 um and using resin coated carrier particles comprising the particles of magnetic substances coated with the resin containing specific fluoro resin in an amount of at least 30% by weight or more, for serving as the above-mentioned carriers.

According to the developing method of the invention, the carrier surfaces are smoothed out, because the carriers forming two-component type developer are resin-coated carriers comprising magnetic particles coated with a resin having a low surface energy as its property. For this reason, there is lime fear that the so-called toner "filming phenomenon" will occur, that is a phenomenon that toner substances adhere to carrier surfaces to hinder the frictional chargeability of the carriers, in a frictional charge between toners and carriers. Therefore, the toners may be endowed stably with a frictional charge having proper polarity and charged volume.

In the case that the carriers forming a two-component type developer are resin-coated carriers comprising magnetic particles coated with resins containing fluoro resins in an amount of not less than a specific proportion, the carrier surfaces are smoothed out, because a fluoro resin is low in critical surface tension as its property. For this reason, there is little fear to occur the so-called toner filming phenomenon, that is a phenomenon that toner substances including, for example, coloring agents such as Carbon Black and so forth, surface releasing agents, etc., adhere to carrier surfaces to hinder the frictional chargeability of the carriers, in a frictional charge between toners and carriers. Therefore, the toners may be endowed stably with a frictionally charge having proper polarity and charged amount. For this reason, the production of weakly charged toners is considerably reduced to hold the toners and carriers stably on a developer transport/carrying member. Resultingly, it is possible to form excellent images without producing any fog and to prevent toners and carriers from flying aboout so as not to contaminate the inside of the apparatus.

The order of frictional chargeability of a fluoro resin is the most negative among resins and, accordingly, the carriers coated with resins containing the fluoro resin are also excellent in negative chargeability. Therefore, in the toners used with the carriers in combination, it is not particularly required to use any charge controller or fine grained additive such as dyes so as to provide the toners with a positive chargeability. Resultingly, the troubles caused when using the charge controllers and the like may be prevented. Besides, the frictional chargeability of toners may be controlled to a considerable degree by selecting a fluoro resin content in the resins for coating carriers. It is, therefore, possible to prepare developers suitable for the developing method of the invention.

Satisfactory fluidity of developers may be obtained even when the carriers are made fine in size, because carrier surfaces are smoothed as mentioned above. Resultingly, a uniform and thin developer layer may be formed on a developer transport/carrying member. Further, the adhesion property of toners to a latent image formed on a latent image carrying member becomes excellent, because the thin developer layer is processed in a developing area where the above-mentioned oscillatory electric field is generated while applying the function of the oscillatory electric field. Resultingly, excellent images may be formed without any uneven imaging and imaging failure.

In addition, the surface releasing property of the carriers becomes excellent, because the carrier surface is smoothed. When a thin developer layer is formed, for example, by bringing a thin layer forming member such as a blade into pressure contact elastically with a developer transport/carrying member, it is possible to prevent carriers from adhering to the thin layer forming member so as to prevent the thickness regulating function of the thin layer forming member from being interfered by the carrier adhesion. Also, when the developer transport member receives a strong pressure by the thin layer forming member, it is possible to prevent carriers from adhering physically and strongly to toners. Therefore, a thin developer layer may stably be formed on the developer transport member. Resultingly, the toner filming phenomenon in which toner substances adhere to carriers may be prevented and an excellent frictional chargeability between toners and carriers may stably be displayed. Thus, sharp images may be formed many times in repetition without any contamination caused in an apparatus by toner and carrier flying.

In the drawings
Fig. 1 is an illustrative sectional view showing an example of a developing unit which may be used in the embodiment of the invention;
Figs. 2(a) and 2(b) are an illustrative perspective view and an illustrative front view each showing an example of a stirring member, respectively;
Fig. 3 is a schematic illustration showing a monochromatic image forming unit;
Fig. 4 is a graph exhibiting the relation between a thin developer layer forming member and a developer transport member and the quantity of developer transported;
Fig. 5 is a schematic illustration showing an example of a multicolor image forming unit;
Fig. 6 is a flow chart for illustrating a multicolor image forming process;
Fig. 7 is a time chart showing the operations of each component of the multicolor image forming unit;
Fig. 8 is a schematic illustration showing another example of the multicolor image forming unit; and
Fig. 9 is a schematic illustration showing an example of a laser optical system.

In this invention, a developer layer having a two-component type developer comprising toners and carriers is formed on a developer transport/carrying member. The developer layer is supplied to a developing area where an oscillatory electric field is generated and an electrostatic latent image on a latent image carrying member is developed. In the above-mentioned developing method, the developer layer formed on the developer transport/carrying member is thin and a resin-coated carrier comprising magnetic particles coated with a resin containing a fluoro resin is used for the carriers.

In the invention, it is required that a developer layer on a developer transport/carrying member is thin. The thickness of the thin layer is preferably not more than 1,000 µm and particularly from 10 to 500 µm.

The development process is carried out in such a manner that a developer layer, which is considerably thin, as mentioned above, is transported into a developing area where an oscillatory electric field is generated so as to bring the developer layer into non-contact with a latent image carrying member and the oscillatory electric field is applied to the developer layer. In the developing area a minimum gap between the latent image carrying member and the developer transport/carrying member (hereinafter called "development gap") is desired to be as narrow as possible, provided that the developer layer may be transported into the developing area so that the developer layer may not come into contact with the latent image carrying member. To be more concrete, the development gap is preferably selected from the range of gap of from 100 to 1,000 µm, for example.

The term "developing area" mentioned herein means an area to which toners transported by a developer transport/carrying member may be able to transfer when an electrostatic latent image on a latent image carrying member receives an electrostatic force.

The term "development gap" means the closest space between a latent image carrying member and a developer transport/carrying member in the above-defined developing area.

The carriers used in the invention are resin-coated carriers comprising magnetic particles coated with a resin containing a fluoro resin in an amount of more than 30% by weight. For example, the thickness of the coated layer is preferably from 0.1 to 10 um on average, more preferably from 0.3 to 4 um and particularly from 0.3 to 2 um. When thinning the coated layer as mentioned above, the developer layer on the developer transport/carrying member may satisfactorily be thinned.

There is no special limitation to the developer transport/carrying members for transporting a thin developer layer to a developing area. The developer transport/carrying members having the same construction as in the conventional types which are capable of applying a bias voltage may also be used. In particular, there may preferably be used those provided with a magnetic roll having a plurality of magnetic poles to the inside of a cylindrical developing sleeve on which a developer layer is carried. In such developer transport/carrying members, as mentioned above, a developer layer carried on the surface of the developing sleeve is transported in undulations like waves by the rotation of the magnetic roll. Thereby, new developers are transported one after another and, in addition, even if there are some irregularities in thickness of the developer layer on the developing sleeve surface, the adverse influence may be compensated by the above-mentioned wave-like undulations, so that no practical problem may be raised.

In the invention, the developer layer formed on a developer transport/carrying member is thinned. In order to develop an electrostatic latent image with an optimum efficiency by making use of the thin developer layer, it is preferred to take the following measures:
(a) A magnetic roll is rotated at a high speed,
(b) An A.C. bias voltage is applied to a developing sleeve,
(c) The development gap, i.e., the closest space between a latent image carrying member and a developing sleeve, is narrowed, and so forth.

In the invention, the non-contact and contact development systems may be used either. Particularly, the non-contact development system is used. The reasons are that the development gap may satisfactorily be narrowed, because the developer layer formed on a developer transport/carrying member is thinned as mentioned before so as to lower the bias voltage required for generating an oscillatory electric field by which toners are properly flown from the developer transport/carrying member to the latent image carrying member in a non-contact developing area, and that there are also the advantages of reducing undesirable toner flying about and preventing the bias voltage from leaking out of the developing sleeve surface, because a satisfactory oscillatory electric field may be generated by the relatively low bias voltage. In addition to the above, in the case of narrowing the development gap, the electric field strength is increased when the field is generated in a developing area by an electrostatic latent image formed-on a latent image carrying member and, resultingly, not only the delicate changes of gradation but fine pattems may excellently be developed.

In the case of thinning the developer layer which is to be carried on a developer transport/carrying member, the amount of toners transported to the developing area is usually reduced and, resultingly, there is the possibility of reducing the amount of toners adhered to an electrostatic latent image on the developer transport/carrying member. To avoid this, it is preferred to rotate the developing sleeve at a high speed so as to increase the amount of toners transported to the developing area On the other hand, when the linear velocity of the developing sleeve exceeds ten times that of the latent image carrying member, the velocity component of the toners transported to the developing area, which velocity component is parallel to the surface subjected to a latent image development of the latent image carrying member, becomes greater and, resultingly, there is the possibility of showing a directivity in development so that the image quality may be worsened.

Taking the above-mentioned circumstances into considerations, it is preferred that toners are present in a proportion of the order of at least 0.04 mg/cm² in a developer layer carried on a developing sleeve

For example, it is preferable to satisfy the following requirements, wherein Vₛ (mm/s) represents the linear velocity of a developing sleeve V_{d} (mm/s) represents the linear velocity of a latent image carrying member, and mₜ (mg/cm²) represents the amount of toners per unit area of a developer layer carried on the developing sleeve:$\left|{\text{V}}_{\text{s}} {\text{/V}}_{\text{d}}\right| {}^{\text{•}} {\text{m}}_{\text{t}} {\text{≧ 0.4 (mg/cm}}^{\text{2}} \text{)}$$\left|{\text{V}}_{\text{s}} {\text{/V}}_{\text{d}}\right| \text{≦ 10}$

In the case of further improving the development efficiency, it is preferable to satisfy the following requirements:$\left|{\text{V}}_{\text{s}} {\text{/V}}_{\text{d}}\right| {}^{\text{•}} {\text{m}}_{\text{t}} {\text{≧ 0.5 (mg/cm}}^{\text{2}} \text{)}$$\left|{\text{V}}_{\text{s}} {\text{/V}}_{\text{d}}\right| \text{≦ 8}$

It was found from the results of experiments that it is more preferable to satisfy the following requirements:$\left|{\text{V}}_{\text{s}} {\text{/V}}_{\text{d}}\right| {\text{Q}}_{\text{t}} {\text{≧ 0.5 (mg/cm}}^{\text{2}} \text{)}$$\left|{\text{V}}_{\text{s}} {\text{/V}}_{\text{d}}\right| {}^{\text{•}} {\text{m}}_{\text{t}} \text{≦ 8}$

In the relation between an amount of toners per unit volume of the toners forming a developer layer carried on a developing sleeve [which is called A (mg/cm³)], it is preferable that a ratio of A/B is from 0.5 to 2.

When performing a development process in accordance with the above-mentioned preferable requirements, the toners contained in a developer layer carried on a developing sleeve may be made to efficiently adhere to an electrostatic latent image formed on a latent image carrying member and a stable development may be made and, resultingly, it is possible to reproduce images having extraordinarily excellent image qualities.

There is no special limitation to the means for forming such a thin developing layer as mentioned before on a developing sleeve, and means having a variety of constitutions may be used. To be more concrete, the examples thereof include a means in which the thickness of a developer layer is regulated by bringing a thin layer forming member such as a blade into pressure contact elastically with the surface of a developing sleeve and, preferably, a means in which the thicknesses of a developer layer are regulated by arranging a regulating plate made of a magnetic substance and a developing sleeve so as to keep a specific gap between them, that is, for example, a means in which the thicknesses of a developer layer are regulated by arranging a magnetic bar close to a developing sleeve and then by generating a rotating magnetic field on the magnetic bar, or other means having been well-known.

From the viewpoint of preventing impurities remaining in a developer, such as dust, fibers, paper dust, aggregates of toners or carriers and the like, from escaping into a developing area, it is particularly preferable to use a thin layer forming member having a pressure plate brought into pressure contact lightly and elastically with a developing sleeve. In this type of thin layer forming members, it is preferable that the edge of the elastic pressure plate is brought into the developing sleeve toward the upper stream side of the rotation of the developing sleeve. with this type of the members, a thin developer layer may be formed by passing a developer through the gap between this elastic pressure plate and the developing sleeve.

Fig. 4 is a diagram illustrating the relation of a gap between the edge of an elastic pressure plate and a developing sleeve (The gap sizes are in proportion to aperture areas) to a quantity per unit area of a developer carried on the developing sleeve, in the case of using the above-mentioned elastic pressure plate.

As is seen from the figure, a quantity per unit area of a developer carried on a developing sleeve shows a stable value regardless of the sizes of a gap, when the gap between the edge of an elastic plate and the developing sleeve exceeds a specific size. In such a stable condition, toners sufficient for developing an electrostatic latent image may be transported into a developing area.

As is understood from the conclusion obtained from Fig. 4, when the gap between the edge of an elastic plate and a developing sleeve is set to not narrower than 0.08 mm, a specific quantity of toners may be transported into the developing area, even if the setting accuracy or the mechanical accuracy varies. In addition, it is more preferable when the gap between the edge of the elastic plate and the developing sleeve is set to not narrower than 0.1 mm, because the stability may be more improved.

However, in order to form a thin developer layer, there is an upper limit for preferably keeping the gap between the edge of the elastic plate and the developing sleeve, that is, a gap of not wider than 5 mm. If exceeding 5 mm, there is some fear of making the thickness of a developing layer uneven.

Fig. 1 is an illustration showing an example of a developing unit suitable for performing the developing method of the invention.

In Fig. 1, reference numeral 20 is a latent image carrying member of, for example, a rotary drum type; 2 is a housing; 3 is a developing sleeve; 4 is a magnetic roll having a magnetic polarity of eight-pole type in total arranged N and S poles alternately around the circumference of the roll; and a developer transport/carrying member is comprised of the developing sleeve 3 and the magnetic roll 4.

Further in Fig.1, 5 is a thin layer forming member; 6 is a member for fixing thin layer forming member 5; 7 is a primary stirring member; 8 is a secondary stirring member; 9 and 10 are the shaft for rotating the above-mentioned stirring members 7 and 8, respectively; 11 is a vessel of replenishing toners; 12 is a roller of replenishing toners; 13 is a developer reservoir; 14 is a bias power source; 15 is a developing area; T is a toner; and D is a developer.

In the above-given developing unit, developer D is well stirred and mixed up in developer reservoir 13 by both of primary stirring member 7 rotating in the direction of the arrow and secondary stirring member 8 rotating in the direction opposite to the rotation of primary stirring member 7 so as to overlap the stirring areas of the both stirring members without colliding against each other and the developer D is then made to adhere to the surface of developing sleeve 3 by the transportation force produced by both of developing sleeve 3 rotating in the direction of the arrow and magnetic roll 4 rotating in the direction opposite to the rotation of the developing sleeve 3.

Plate-like thin layer forming member 5 comprising an elastic material brings one side of the plate close to the edge into pressure contact with the surface of developing sleeve 3. This thin layer forming member 5 is held by fixing member 6 extended from housing 2. By this thin layer forming member 5, the thicknesses of a developer layer being transported into developing area 15 are regulated to thin the developer layer.

The developer layer thinned in this manner is transported into developing area 15 as the layer is facing to an electrostatic latent image formed on latent image carrying member 20 rotating in the direction of the arrow, preferably through a narrow gap, so to say, so as not to come into contact with each other. In the developing area 15, while the thin developer layer is being subjected to an oscillatory electric field generated by bias power source 14 containing A.C. components, only the toners held in the developer layer selectively and statically adhere to the electrostatic latent image, so that a toner image is formed.

The thickness of the developer layer may be measured in the following manner, for example. With a "Nikon Profile Projector" (manufactured by Nippon Kogaku Co.), the position of the image of a developing sleeve projected on a screen and the position of the image of a thin developer layer formed on the developing sleeve projected on the screen are compared with each other to obtain the thickness of the developer layer.

Thin layer forming member 5 may be made of, for example, a magnetic or non-magnetic metal, a metal compound, a plastic, rubber and so forth. This member 5 is endowed with elasticity by fixing one end of the member 5 with fixing member 6. It is preferable that the thickness of this member 5 is very thin and uniform in thickness, that is from 50 to 500 µm.

The amount of carrier transported is regulated in such a manner that the above-mentioned thin layer forming member 5 brings one side close to the edge thereof into contact elastically with developing sleeve 3 and, preferably, the carriers may be passed one after another through the contact position of the thin layer forming member 5 with developing sleeve 3. The impurities remaining in developer D, aggregates of carriers or toners and so forth are prevented from stealing into developing area 15 by the thin layer forming member 5. Therefore, every developer layer transported into developing area 15 becomes thin, uniform and stable in thickness.

The developing method of the invention uses a resin-coated carrier which is, coated with a resin containing a fluoro resin in a specific proportion or more. Therefore, the surface of the carrier is excellently smoothed even if the carrier is small-sized, because of the coated layer. The fluidity of the carrier is thereby improved. Accordingly, the thickness regulating function of the thin layer forming member 5 is satisfactorily displayed and, resultingly, every developer layer transported into developing area 15 may be satisfactorily uniformed and thinned in thickness. Further, the surface lubricity of the carrier is also excellent because of the coated layer. Therefore, the so-called filming phenomenon, that is, an adhesion of toner substances to carriers, may be prevented, even if the developer layer is applied with a strong pressure by thin layer forming member 5.

The amount of developer transported into developing area 15 may satisfactorily be controlled by changing the pressure and contact angles applied from thin layer forming member 5 to developing sleeve 3.

In toners and carriers forming a developer, it is generally advantageous that they are small-sized, because an image obtainable is high in resolving power and excellent in gradation reproduction. For example even in the case of using a two-component type developer comprising toners having a weight average particle size of not larger than 5 µm and carriers having a weight average particle size of not larger than 50 µm and further not larger than 30 µm, any impurities, particle aggregates and so forth may automatically be removed from the developer so as to form uniformed and thinned developer layer. In addition, even in the case of using a developer comprising toners and small-sized carriers having a weight average particle size of the same order as that of the toners, any impurities may be prohibited from stealing into the resulting developer layer by thin layer forming member 5 similar to the above-mentioned example, so that a uniformed and thinned developed layer may be formed.

On the other hand, in order to prevent carriers from adhering to latent image carrying member 20, it is preferable to use carriers having relatively larger particle size, because the carriers may be attracted to the surface of the developer transport/carrying member by an intensive magnetic force.

Taking the above-mentioned circumstances into consideration, it is advantageous to use a carrier having a weight average particle size of the order of from 50 to 100 µm. In this case, a satisfactorily uniform and thin developer layer may be formed by thin layer forming member 5 and a carrier may also satisfactorily be prevented from adhering to latent image carrying member 20. In contrast to the above, when using carriers having an excessively large weight average particle size, brush-like ears (i.e., a magnetic brush) of the carriers held in a developer layer are heightened and the layer is made coarse, so that the developability is lowered.

In order to make carriers receivable an intensive magnetic force,even if they are small-sized, the magnetization of the carriers is preferably from 10 to 200 emu/g, more preferably from 10 to 100 emu/g and, particularly from 15 to 30 emu/g. If the magnetization of the carriers is too little, there may be some instance where none of excellent magnetic brushes may be formed. If the magnetization is too great, there may be some instances where an oscillatory electric field may not function well, so that an excellent image may hardly be formed.

Figs. 2(a) and 2(b) are a perspective view and a front view each for illustrating an example of the detailed unit structure of stirring members 7 and 8.

In the drawings, 7a, 7b and 7c are stirring blades of primary stirring member 7 and 8a, 8b and 8c are the stirring blades of secondary stirring member 8, respectively. There is no special limitation to the detailed forms of the blades, however, it is preferable to select a blade form from the square, tabular, elliptic and the like forms. These stirring blades are arranged at an angle and/or position different from each other blades and fixed to rotating shafts 9 and 10, respectively. These stirring members 7 and 8 are so arranged as to overlap each other member in a stirring area without colliding with the other blades. In Fig. 1, therefore, stirring may satisfactorily be performed in the direction from right to left At the same time, each stirring blade is slanted to the corresponding rotating shaft and fixed. In Fig. 1, therefore, stirring may also satisfactorily be performed in the direction of back and forth. Accordingly, toners T are replenished from toner replenishing vessel 11 through replenishing roller 12 so that they are uniformly mixed up with developer D within a short time.

Toners and carriers are frictionally charged well by the above-mentioned stirring members 7 and 8 and the resulting developers are allowed to adhere to and be held on developing sleeve 3 by magnetic force, and a thin developer layer is then formed by thin layer forming member 5.

While being transported toward a specific direction by the rotation of the developing sleeve 3, the thin developer layer receives a magnetic bias having an oscillatory component and derived from the reverse rotation of the magnetic roll 4 and performs a single motion, such as rolling, on the developing sleeve 3. Accordingly, the toner particles satisfactorily adhere to an electrostatic latent image formed on the latent image carrying member 20,especially if the thin developer layer transported to the developing area receives the influence of the oscillatory electric field on a non-contact basis in relation to the electrostatic latent image.

According to the invention, the thickness of developer layer is favorably set extremely small, or more specifically, at 10 to 500 µm. This arrangement enables to narrow the development gap between the latent image carrying member 20 and the developing sleeve, for example, to 500 µm, and accordingly, ensures development in compliance with the so-called noncontact developing system.

Such a narrower development gap enhances the electric field strength in the developing area 15. This in turn enables satisfactory development operation even if the bias voltage applied onto the developing sleeve 3 is smal!er, and, advantageously, reduces the leakage of bias voltage, and other disadvantages. Furthermore, the resultant greater contrast in the electrostatic latent image generally improves the resolution and quality of an image obtainable from the development operation.

with this example, when the development is effected by the non-contact development system, only the toner powder is selectively allowed to jump to an electrostatic latent image to be developed. This arrangement in turn prevents the carrier powder from adhering to the electrostatic latent image area, thus precluding the possibility of the deteriorated image quality. Additionally, since a magnetic brush never rubs the electrostatic latent image area, and, naturally does. not damage the surface of electrostatic image carrying member or cause a brush pattern phenomenon, resulting in improved image resolution and gradation reproducibility, and a sufficient amount of toner being adhered to the electrostatic latent image. Furthermore, the developing method of the invention may be favorably used for a multicolor development system in which the development process is repeatedly effected on an latent image carrying member where a toner image is formed.

The developer used in embodying the invention is a two-component developer comprising a toner, as well as a resin-coated carrier composed of magnetic particles each of which being coated with resin involving fluoro resin in an amount of at least 30 % by weight.

The toner comprises fine particles each composed of binder resin containing a toner component such as a coloring agent.

The preferred binder resins used for toner include polyester resin, styrene-acryl resin, and the like.

The polyester resin favorably used as the binder resin of toner is prepared by the condensation polymerization of alcohol monomer and carboxylic monomer. The examples of such an alcohol monomer are as follows: diols such as ethylene glycol, diethylene glycol, triethylene glycol, 1,2-propylene glycol, 1,3-propylene glycol, 1,4-butanediol, neopentyl glycol, 1,4-butenediol and the like; etherified bisphenols such as 1,4-bis(hydroxymethyl) cyclohexane, bisphenol A, hydrogenated bisphenol A, polyoxyethylene bisphenol A, polyoxypropylene bisphenol A and the like; other bivalent alcohol monomers. The examples of such a bivalent carboxylic monomer are as follows; maleic acid, fumaric acid, methaconic acid, citraconic acid, itaconic acid, glutaconic acid, phthalic acid, isophthalic acid, cyclohexanedicarboxylic acid, succinic acid, adipic acid, sebatic acid, malonic acid; anhydrides, lower alkyl esters, and linolenic dimers of these acids; other bivalent organic acid monomers.

As a polyester resin favorably used as the binder resins of toner, polymers having multifunctional monomeric components, larger than trifunctional ones, are also favorably used in addition to the polymers comprising the above bifunctional monomers. The examples of multivalent alcohol monomers, or the above multifunctional monomers, whose valence being larger than trivalence, are as follows: sorbitol, 1,2,3,6-hexanetetrol, 1,4-sorbitan, pentaerythritol, dipentaerythritol, tripentaerythritol, saccharose, 1,2,4-butanetriol, 1,2,5-pentanetriol, glycerol, 2-methylpropanetriol, 2-methyl-1,2,4-butanetriol, trimethylolethane, trimethylolpropane, 1,3,5-trihydroxymethylbenzene, and the like.

The examples of multivalent carboxylic monomers whose valence being larger than trivalence, are as follows: 1,2,4-benzenetricarboxylic acid, 1,3,5-benzenetricarboxylic acid, 1,2,4-cyclohexanetricarboxylic acid, 2,5,7-naphthalenetricarboxylic acid, 1,2,4-naphthalenetricarboxylic acid, 1,2,4-butanetricarboxylic acid, 1,2,5-hexanetricarboxylic acid, 1,3-dicarboxyl-2-methyl-2-methylenecarboxylpropane, tetra (methylenecarboxy)methan, 1,2,7,8-octanetetracarboxylic acid, empoltrimer acid; anhydrides of these acids; and others.

As the above-mentioned styrene-acryl resin, the resins not only having an Mw/Mn ratio, which is a ratio between weight-average molecular-weight Mw and number-average molecular-weight Mn, of more than 3.5 but containing α, β-unsaturated ethylene monomer, which are disclosed for example in JP-A-134652/1975, as a component are favorably used. The typical examples of such an α, β-unsaturated ethylene monomer are as follows: aromatic vinyl monomers such as styrene, o-methylstyrene, p-methylstyrene, α-methylstyrene, p-ethylstyrene, 2,4-dimethylstryrene, p-n-butylstyrene, p-tert-butylstyrene, p-n-hexylstyrene, p-n-oxtylstyrene, p-n-nonylstyrene, p-n-decylstyrene, p-n-dodecylstyrene, p-methoxystyrene, p-phenylstyrene, p-chlorostyrene, 3,4-dichlorostyrene and the like; acrylic esters such as methyl acrylate, ethyl acrylate, n-butyl acrylate, isobutyl acrylate, propyl acrylate, n-octyl acrylate, dodecyl acrylate, lauryl acrylate, 2-ethylhexyl acrylate, stearyl acrylate, 2-chloroethyl acrylate, phenyl acrylate, methyl α-chloroacrylate and the like; methacrylic esters such as methyl methacrylate, ethyl methacrylate, propyl methacrylate, n-butyl methacrylate, isobutyl methacrylate, n-octyl methacrylate, dodecyl methacrylate, lauryl methacrylate, 2-ethylhexyl methacrylate, stearyl methacrylate, phenyl methacrylate, dimethylaminoethyl methacrylate, diethylaminoethyl and the like; vinyl halides such as vinyl chloride, vinylidene chloride, vinyl fluoride and the like; nivyl esters such as vinyl acetate, vinyl propionate, vinyl benzoate, vinyl butyrate and the like; and others.

The values of number-average molecular-weight Mn and weight-average molecular-weight Mw in a specific polymer may be measured by various methods. Though the measured results differ depending upon the measuring method, the number-average molecular-weight Mn as well as the weight-average molecular-weight Mw in this specification are defined as the values determined by the following method.

In other words, each of these values is a value determined by a gel permeation chromatography with the following conditions; a solvent (tetrahydrofuran) is allowed to flow at a rate of 1.2 ml per minute with a temperature of 40° C, whereby 3 mg tetrahydrofuran solution of a density 0.2 g/20 ml containing a sample is added for the measuring operation, In determining the molecular weight of a sample, measuring, conditions are selected so that the counted number of the molecular weight of the sample provides a linear relation with the logarithmic numbers on the analytical curve formed from the measuring results with various types of monodispersion polystyrene reference samples.

Additionally, the reliability of the measuring result is confirmed when a NBS 708 polystyrene reference sample satisfies the following expressions under the above-mentioned measuring conditions.${\text{Weight-average molecular-weight Mw = 28.8 x 10}}^{\text{4}}$${\text{Number-average molecular-weight Mn = 13.7 x 10}}^{\text{4}}$

As a GPC column used for this purpose, any columns may be used as for as they satisfy the above conditions. More specifically, a TSK_GE, GMH (manufactured by Toyo Soda Mfg. Co., Ltd.) or the like may be used.

A preferred binder resin used for toner has a softening point Tsp of 80 to 150° C, or, more specifically, 100 to 140° C. The glass transition point Tg of the similar resin is favorably 40 to 80°C, or in particular, 50 to 70°C. By using such a binder resin, a toner having both low-temperature fixing property and excellent antiblocking property is obtained, and accordingly, a satisfactory developing operation is achieved, enabling a final image to be rapidly formed.

Unless otherwise specified, the softening point Tsp refers to a temperature determined in the following manner: using a flow tester Model CFT-500 manufactured by Shimazu Seisakusho Ltd., the measurement was recorded with measuring conditions of 20 kg/cm² load, 1 mm nozzle diameter, 1 mm nozzle length, 80°C pre-heating for 10 minutes, 6° C/min heating rate, and 1 cm³ (weight represented by intrinsic specific gravity x 1 cm³), wherein, by assuming the height of S curve in the characteristic curve (softening fluidization curve) representing the correlation between the amount of plunger drop in the flow tester and the corresponding temperature is h, the softening point is determined by reading a temperature corresponding to h/2.

The glass transition point is a value determined in the following manner: using a differential scanning calorimeter Model Low-temperature DSC manufactured by Rigaku Denkisha Co., Ltd., a measuring operation is performed at a heating rate of 10°C/min, whereby the glass transition point is read from the temperature on an intersection, in a DSC thermogram, between the extension of baseline below the glass-transition point and the tangent line representing a maximum slope from the initial rising portion to summit of a peak.

The toner used in the invention comprises binder resin particles containing a coloring agent, as well as other toner component added in compliance with a requirement.

The examples of useful coloring agent are as follows: Carbon Black, Nigrosine Dye (C.I. No. 50415B), Aniline Blue (C.I: No. 50405), Chalcoil Blue (C.I. No. Azoic Blue 3), Chrome Yellow (C.I. No. 14090), Ultramarine Blue (C.I. No. 77103), DuPont Oil Red (C.I. No. 26105), Quinoline Yellow (C.I. No. 47005), Methylene Blue Chloride (C.I. No. 52015), Phthalocyanine Blue (C.I. No. 74160), Malachite Green Oxalate (C.I. No. 42000), Lamp Black (C.I. No. 77266), Rose Bengal (C.I. No. 45435), and mixtures involving any of the above agents, and others.

Sufficient proportion of such a coloring agent is favorably incorporated into a toner so as to form a satisfactorily dense image. The amount of such agent is usually 1 to 20 parts weight per 100 parts weight toner.

To prevent the filming of toner substance on a carrier, various surface releasing agents are favorably incorporated into the toner.

The examples of such a useful surface releasing agent include polyolefin, metal salt of aliphatic acid, aliphatic ester, partially saponified aliphatic ester, higher alcohol, fluid or solid paraffin wax, amide wax, multivalent alcohol ester, silicone varnish, aliphatic fluoro carbon, and the like. Among these examples, those preferred have a softening point, measured by a ring and ball test specified in JIS K2531-1960, of 80 to 180° C, in particular 70 to 160° C. These surface'releasing agents may be singly used, or more than two of them may be combinedly used.

The examples of above-mentioned useful polyolefin include resins such as polypropylene, polyethylene, polybutene and the like.

The examples of above-mentioned metal salt of aliphatic acid are as follows: salts of maleic acid and a metal such as zinc; magnesium, calcium and the like; salts of stearic acid and a metal such as zinc, cadmium; barium, lead, iron nickel, cobalt, copper aluminum, magnesium, and the like: lead salt of dibasic stearic acid; salts of oleinic acid and a metal such as zinc, magnesium, iron, cobalt, copper, lead, calcium and the like; salts of palmitic acid and a metal such as aluminum, calcium and the like; lead caprate, lead capronate, metal salts of linoleic acid and a metal such as zinc, cobalt and the like; salts of ricinoleic acid and a metal such as zinc, cadmium and the like; and the mixture of these salts.

The examples of the above-mentioned useful aliphatic ester include ethyl maleate, butyl maleate, methyl stearate, butyl stearate, cetyl palmitate, ethylene glycol montanate and the like

As the above partially saponified aliphatic ester, for example, a montanic ester whose calcium area is saponified may be used.

The examples of the above-mentioned useful higher aliphatic acid include dodecanic acid, lauric acid, myristic acid, palmitic acid, stearic acid, oleic acid, linolic acid, ricinoleic acid, arachic acid, behenic acid, lignoceric acid, ceracholeic acid and the like, and a mixture of these acids.

The examples of the above-mentioned useful higher alcohol include dodecyl alcohol, lauryl alcohol, myristyl alcohol, palmityl alcohol, stearyl alcohol, aralkyl alcohol, behenyl alcohol and the like.

The examples of the above-mentioned useful paraffin wax include natural paraffin, microcrystalline wax, synthetic paraffin, chlorinated hydrocarbon and the like.

The examples of the above-mentioned useful amide wax include amide stearate, amide oleinate, amide palmitate, amide laurate, amide behenate, methylenebisstearoamide, ethylenebisstearoamide and the like.

The examples of the above-mentioned useful alcohol ester include glycerol stearate, glycerol ricinolate, glycerol monobehenate, sorbitan monostearate, propylene glycol monostearate, sorbitan triolate and the like.

The examples of the above-mentioned useful aliphatic fluoro carbon include lower polymers such as ethylene tetrafluoride and propylene hexafluoride, and a fluorine-containing surface active agent disclosed in JP-A-124428/1978, and other agents.

The proportion of these surface release agents to be used is favorably 1 to 10 part weight per 100 parts weight binder resin.

Other useful toner components are as follows: fluidizing agents such as fine silica powder, fine titania powder, fine alumina powder and the like; abrasive powder such as cerium oxide; lubricants such as zinc stearate and the like; charge controlling agents such as pigment or dye; and others.

The preferred toner used in the invention has a weight-average particle size of less than 20 µm, in particular, 1 to 15 µm. The use of a toner having such a preferred weight-average particle size enables an image having extremely good image quality to be formed. In contrast, the use of a toner having an excessively large weight-average particle size readily decreases the image resolution and may sometimes decrease the gradation reproducibility. At the same time, the use of a toner having an excessively small weight-average particle size may cause the toner to fly around in an image forming apparatus, and this in turn may sometimes decrease the sharpness of resultant image.

According to the invention a carrier composing a two-component developer together with a toner is, as mentioned previously, a resin-coated carrier whose individual particles comprise a magnetic particle coated with a resin containing fluoro resin in an amount of at least 30% by weight thereof.

The scope of fluoro resins used for forming the coating layer of carrier is not specifically limited, however, the fluoro resin is one capable of being dissolved in solvent, and being applied onto the surface of magnetic particles by a conventional coating method.

More specifically, the following are used.
(1) Vinylidene fluoride-tetrafluoroethylene copolymer,
(2) Polymer comprising a vinyl ether monomer represented by the following general formula and having a substituent in the position of a fluorine atom in the side chain wherein R_{f} represents an alkyl group or aralkyl group substituting more than one fluorine atom.
(3) Polymer comprising a vinyl ketone monomer represented by the following general formula wherein R_{f} represents an alkyl group or aralkyl group substituting more than one fluorine atom.
(4) Blend polymer comprising more than two of the resins correspondingly represented by the above formulas (1) through (3).

The fluoro resin used to form the coating layer of carrier is prepared by singly or combinedly using the above-described fluoro resins or a resin having not only the above fluoro resin but another resin may be used for this purpose. Such another resin is favorably one having a high compatibility with a fluoro resin. The examples of such a resin include an acryl resin, styrene resin, epoxy resin, urethane resin, polyamide resin, polyester resin, acetal resin, polycarbonate resin, phenol resin, vinyl chloride resin, vinyl acetate resin, cellulose resin, polyolefin resin, copolymers of these resins, blend results of these resins, and others.

The content of fluoro resin in the coating resin is at least 30 weight%, or more favorably, 40 to 100 weight%, or most favorably 50 to 100 weight% Less than 30 weight% of fluoro resin content does not fully provide the favorable property of fluoro resin, often resulting in unstable triboelectric charging characteristic.

With a resin-coated carrier used in the invention, the magnetic particle serving as a core being coated with a resin is a particle made of a substance which, is strongly magnetized in the direction of magnetic field. The examples of such a substance are as follows: metals showing ferromagnetism such as ferrite, magnetite, as well as iron, nickel, cobalt and the like; alloys or compounds involving these metals; alloy not having ferromagnetic element but being endowed with ferromagnetism by an appropriate heat-treatment, and being typified by Heusler alloys such as manganese-copper-aluminum alloy, manganese-copper-tin and the like; chromium dioxide and the like.

The term "ferrite" is a general term of a magnetic oxide involving iron and is not limited only to a Spinel structure ferrite represented by the formula MO.Fe₂O₃ (M represents a bivalent metal atom). Capable of being arbitrarily providing various magnetic characteristics by varying the composition of contained metal components, a ferrite is especially advantageous to prepare a carrier which best suits the object of the invention. Additionally, being made of oxidant, the ferrite powder has a specific gravity much smaller than metal powder such as iron powder or nickel powder. This feature allows easy mixing and blending with a toner, and advantageously contributes to the uniformity of toner concentration in the developer as well as to the optimization of triboelectrical potential formed in toner powder. A further advantage is that, since having a resistivity of 10⁸ to 10¹²Ω.cm, which is greater than that of iron powder, nickel powder or cobalt powder, the ferrite powder provides an insulative carrier satisfactorily used in a developing method in which a high bias voltage is applied to the developing gap, even when the layer thickness of resin forming the surface of the carrier particle is extremely small, approximately 0.5 µm.

In relation to the 1000 Oe external magnetic field, the above-mentioned ferrite favorably has a saturated magnetization of 10 to 40 emu/g and a coercive force of 0.1 to 100 Oe. Furthermore, the ferrite favorably has a resistivity of 1 x 10⁶ to 1 x 10¹¹Ω.cm, a specific gravity of 4.0 to 5.5, and a porosity of 1.0 to 10%.

In preparing a resin coated carrier, the coating layer is formed in the following steps. A solution prepared by dissolving fluoro resin, and, if necessary, another resin, in a solvent is applied on the surface of individual magnetic particles by a dipping method, spray method, fluidized bed method or the like, whereby usually by heating, the solvent is allowed to vaporize and the solution is allowed to dry, then during or after the drying, the coat layer is allowed to set.

Into the coating solution to form the coating layer may be added other additives in compliance with a requirement. A solvent being used for this purpose is not specifically limited, as far as a silicone resin, fluororesin, and another additional resin can be dissolved in such a solvent. However, the typical examples of such a solvent are as follows: aromatic hydrocarbons such as toluene, xylene and the like; ketones such as acetone, methylethyl ketone; tetrahydrofuran; dioxane; higher alcohol; and mixed solvents involving any of the above solvents.

The preferred heating temperature necessary for setting a coating layer comprising a resin containing fluoro resin is usually 100 to 350° C. To accelerate the drying or setting, a dryer or setter composed of, for example, an organic metal salt such as zinc octylate, dibutyl zinc oxide or the like may be used.

The preferred thickness of the formed resin coating-layer containing fluoro resin is, for example, 0.1 to 10 µm, and more specifically, 0.3 to 4 µm, and most specifically, 0.3 to 2 µm.

The individual particles of resin-coated carrier used in the invention are favorably spherical-shaped and have a weight-average particle size of less than 100 um, and more favorably, 5 to 50 µm. The use of a resin-coated carrier having such a favorable weight-average particle size improves the image resolution as well as the gradation reproducibility. The use of a carrier having an excessively large weight-average particle size may sometimes make it difficult to form a thin developer layer on a developer bearing/carrying member, and possibly resulting in the deteriorated developability and decreased image quality. In contrast, the use of a carrier having an excessively small weight-average particle size may sometimes deteriorate the developability, triboelectrical charging property, fluidity and the like, and may cause the carrier to fly around in an image forming apparatus.

A resin-coated carrier used in the invention is an insulative carrier having a resistivity of more than 10⁸Ω.cm, favorably, more than 10¹³Ω.cm, and more favorably, more than 10¹⁴Ω.cm. The use of such a highly insulative carrier satisfactorily prevents, in the course of developing, a potential from being injected by a bias voltage and resulting in a filming of carrier on the surface of a latent image carrying member, or a potential to form an electrostatic latent image from being eliminated.

Incidentally, the weight-average particle sizes of toner and carrier are values determined with a Coulter Counter manufactured by Coulter Ltd.

The resistivities of magnetic particles as well as resin-coated carrier particles are determined by the following procedure: sample particles are poured into a container having a cross-sectional area of 0.50 cm² and tamped down, then a load of 1 kg/cm² is applied onto the tamped sample particles so as to make the thickness of sample to be approximately 1 mm, whereby an electrical field of 102 to 105 V/cm is applied to between the load and a bottom electrode and the value of current flowing is measured.

In preparing a two-component developer used in the invention, the preferred blending ratio between toner and carrier is a ratio where the total surface area of toner is approximately the same as the similar area of carrier. For example, if the weight-average particle size of toner is 10 um and the weight-average particle size of carrier is 20 um, the preferred toner concentration (weight ratio per total developer) is 5 to 40 weight%, in particular, 8 to 25 weight%. More specifically, unlike a conventional developer comprising large-sized carrier particles whose individual surface being covered with a multiplicity of toner particles, it is advantageous to prepare the two-component developer used in embodying the invention by blending a toner and a fine particle carrier whose particle size being approximately the same as the toner at a ratio where the total surface areas of carrier and toner are approximately the same with each other.

### [Typical Examples]

The typical examples are hereinafter described, in order to further describe the invention.

First, an example where a resin-coated carrier comprising magnetic particles coated with silicon resin-containing resin is described below, which does not form part of the invention.

### (Example 1)

Fig. 3 is an explanatory diagram schematically illustrating one example of image forming apparatus being used in embodying the developing method of the invention. The move of a draft table causes the optical draft image formed by an illuminating light source 21 to be focused on a latent image carrying member 20 via a mirror 22 and a lens 23, and an electrostatic latent image corresponding to an original draft is formed on the latent image carrying member 20. A developing unit A has a constitution, for example, shown in Fig. 1. The electrostatic latent image formed on the latent image carrying member is developed by the developing unit A to form a toner image.

A toner image obtained in such a manner is transferred onto a recording paper P with a transfer electrode 29 after being electrically neutralized for easy transfer by an exposure lamp 28. The recording paper P is separated by a separation electrode from the latent image carrying member 20 and is fixed with a fixer 31 to form a fixed image. At the same time, the latent image carrying member 20 is electrically neutralized by a neutralization electrode 32 and its surface is cleaned by a cleaning mechanism 33.

The cleaning mechanism 35 in this example has a cleaning blade 34 for scraping off toner. Toner particles scraped off by the blade 34 are collected by a roller 36.

Using such an image forming apparatus and developing method, the following test procedure was exercised by actually conducting image forming operation.

### Preparation of resin-coated carrier

### (1) Carrier A

With a fluidized-bed equipment 100 parts spherical copper-zinc ferrite particles having a weight-average particle size of 35 um (manufactured by TDK Corporation) were coated with 25 parts condensation-reaction type silicone resin solution SR-2411 (manufactured by Toray Silicone Co., Ltd.) at a temperature of 80°C, and were further heat-treated at a temperature of 200°C for one hour to obtain a carrier having individual particles being coated with a silicone resin layer. The coating layer has a thickness of approximately 1 um. The carrier was designated carrier A.

The properties of the carrier A were as follows:

| | |
|---|---|
| Weight average particle size | 42 µm |
| Magnetization (Measured magnetic field: 1000 Oe) | 20 emu/g |
| Resistivity | more than 10¹⁴ Ω.cm |
| Specific gravity | 4.9 g/cm³ |

### (2) Carrier B

A carrier having particles individually being coated with a 1 um thick silicone resin layer was prepared in a manner identical to that of carrier A except that silicone resin solution SR-2410 was used in the place of silicone resin solution SR-2411. This carrier was designated carrier B. The properties of the carrier B were as follows:

| | |
|---|---|
| Weight-average particle size | 35 µm |
| Magnetization (Measured magnetic field: 1000 Oe) | 16 emu/g |
| Resistivity | 10¹⁴ Ω.cm |
| Specific gravity | 4.8 g/cm³ |

### (3) Carrier C

A carrier having particles individually being coated with a 1 um thick silicone resin layer was prepared in a manner identical to that of carrier A except that thermosetting silicone resin solution (manufactured by The Sin-Etsu Chemical Co., Ltd.) was used in the place of silicone resin solution SR-2411. This carrier was designated carrier C.

The properties of the carrier C were as follows:

| | |
|---|---|
| Weight average particle size | 42 µm |
| Magnetization (Measured magnetic field: 1000 Oe) | 14 emu/g |
| Resistivity | more than 10¹⁴ Ω.cm |
| Specific gravity | 4.8 g/cm³ |

### (4) Comparison carrier a

A carrier comprising copper-zinc ferrite particles identical to those of carrier A was designated comparison carrier a.

The properties of the comparison carrier a were as follows:

| | |
|---|---|
| Weight-average particle size | 40 µm |
| Magnetization (Measured magnetic field: 1000 Oe) | 18 emu/g |
| Resistivity | 4 × 10¹⁰ Ω.cm |
| Specific gravity | 5.2 g/cm³ |

### (5) Comparison carrier b

A carrier having particles individually have a coating layer of 1 µm thick styrene was prepared in a manner identical to that of carrier A except that toluene solution (solid content 10 weight%) containing styrene resin (weight-average molecular weight Mw, 71,000; number-average molecular weight Mn, 32.000; glass transition point Tg, 125°C) was used in the place of silicone resin solution SR-2411. This carrier was designated comparison carrier b.

The properties of the comparison carrier b were as follows:

| | |
|---|---|
| Magnetism (Measured magnetic field: 1000 Oe) | 20 emu/g |
| Resistivity | more than 10¹⁴ Ω.cm |
| Specific gravity | 4.9 g/cm³ |

### (6) Comparison carrier c

A carrier having particles individually being coated with a 1.5 um thick methyl methacrylate resin layer was prepared in a manner identical to that of carrier A except that toluene solution (solid content, 10 weight%) containing methyl methacrylate resin (weight average molecular Mw, 73,000; number average molecular Mn, 33,000; glass transition point Tg:-121° C) was used in the place of silicone resin solution SR-2411. This carrier was designated comparison carrier c.

The properties of the comparison carrier c were as follows:

| | |
|---|---|
| Weight-average particle size | 40 µm |
| Magnetization (Measured magnetic field: 1000 Oe) | 20 emu/g |
| Resistivity | more than 10¹⁴ Ω.cm |
| Specific gravity | 4.8 g/cm³2 |

### Preparation of toners

### (1) Black toner A

With a Henschel mixer, 100 parts weight polyester resin (UXK-120 P, manufactured by Kao Soap Co., Ltd.) and 3 parts weight polypropylene (Viscol 660 P, manufactured by Sanyo Kasei Kogyo Co., Ltd.) and 10 parts Carbon Black (Mogal L, manufactured by Cabot) and 2 parts weight charge controlling agent (Bontron E-82, manufactured by Orient Chemicals Co., Ltd.) were mixed, then thoroughly kneaded with a triple-roller at a temperature of 140° C. Further, the mixture, after cooled and crushed, was pulverized with a jet mill and classified to prepare black toner powder having a particle size distribution of 5 to 25 um and a weight-average particle size of 11 µm.

To 100 parts weight of the black toner powder, 0.5 parts weight hydrophobic fine silica particles (R-812, manufactured by Nippon Aerozyl Co., Ltd.) was added, then thoroughly blended by a Henschel mixer to prepare black toner. This toner was designated black toner A. The static bulk density of the black toner A was 0.44 g/cm³.

### (2) Yellow toner B

A yellow toner was prepared in a manner identical to that of black toner A except that yellow pigment, Pigment Yellow, was used in the place of Carbon Black. This toner was designated yellow toner B. The static bulk density of the yellow toner B was 0.44 g/cm³.

### (3) Magenta toner C

A magenta toner was prepared in a manner identical to that of black toner A except that magenta pigment, Permanent Carmine F-5B, was used in the place of Carbon Black. This toner was designated magenta toner C. The static bulk density of the magenta toner C was 0.45 g/cm³.

### (4) Cyan toner D

A cyan toner was prepared in a manner identical to that of black toner A except that cyan pigment, Copper Phthalocyanine, was used in the place of Carbon Black. This toner was designated cyan toner D. The static bulk density of the cyan toner D was 0.44 g/cm³.

### Preparation of developers

The above-mentioned carriers A through C were independently combined with the black toner A to prepare developers 1 through 3 individually having a toner concentration of 10 weight%. At the same time, the above-mentioned comparison carriers a through c were also combined with the black toner A to correspondingly prepare comparison developer 1 through 3 individually having a toner concentration of 10 weight%.

Additionally, yellow toner B, magenta toner C and cyan toner D were independently combined with carrier A to correspondingly prepare color developers 1 through 3 individually having a toner concentration of 12 weight%.

### Test 1 by actual copying operation

Using each of these developers, a test was performed by executing copying operation, in accordance with the developing process based on the below specified developing conditions, for 30,000 sheets, whereby the triboelectricity on toner, fog, adhesion of carrier on a latent image carrying member, imaging failure, and uneven imaging were evaluated at the first and 30000th formed images. The results are listed in Table 1 shown later.

[Developing conditions (normal developing)]
o Latent image carrying member: 100 mm dia, drum type photosensitive member made of selenium
o Linear velocity: 100 mm/sec
o Surface potential: + 800 V (image area) to + 50 V (non-image area)
o Diameter of developing sleeve: 25 mm
o Linear velocity of developing sleeve: 250 mm/s (forward direction)
o Total number of poles on magnetic roll: 8 poles
o Rotational speed of magnetic roll: 1200 rpm
o Thin layer forming member: 3 mm thick resilient plate made of urethane rubber, being pressed on the surface of developing sleeve
o Development gap: 500 µm
o Thickness of developer layer: 400 µm (maximum value)
o Toner content in developer: 10 weight%
o Toner content in developer layer formed on developing sleeve: 0.3 mg/cm²
o DC bias voltage: 50 to 200 V
o AC bias voltage: 1.0 to 2 kV (frequency, 3 kHz; peakpeak value)

The methods of evaluation were as follows:

### Triboelectricity

Measured by a known blow-off method.

### Fog

A fixed image was inspected with human eye.

### Carrier adhesion on latent image carrying/transporting member

The surface of latent image carrying/transporting member was inspected with human eye.

### Imaging failure

A fixed image was inspected with human eye.

### Adhesion of toner material to the surface of carrier (toner spent)

Judged by inspecting carrier particles with a scanning electron microscope.

As can be understood from the results listed in Table 1, when executing the developing method of the invention with any of the developers 1 through 3, the toner demonstrated a proper triboelectricity, and a sharp image featuring high-resolution as well as excellent gradation reproducibility is formed without accompanying any of fog, carrier adhesion of the image carrying member, imaging failure, and uneven imaging.

With a fluctuation in toner triboelectricity being small, the developing method using any of the developers 1 through 3 provides a sharp image, whose quality is comparable to that of the first copied image, even after 30000 sheet-copying operation. Additionally, inspection of the contamination in an image forming apparatus confirmed only an extremely limited contamination with toner and carrier. This is because the silicone resin to form the coating layer of the carrier has a smaller critical surface tension when compared to a resin used to prepare a comparison carrier, and accordingly, the toner substance does not easily adhere to the surface of individual carrier particles. Furthermore, the developing effect of bias voltage was satisfactorily demonstrated.

In contrast, the comparison developer 1 incurred a smaller triboelectricity even in the initial stage of continuous 30000 sheet copying operation, and an obtained image was not sharp, showing considerable fog, imaging failure and uneven imaging. Also, the carrier adhesion on the latent image carrying member was found. In addition, the above problems further deteriorated after the completion of 30000-sheet copying operation, because of further decreased toner triboelectricity. Also, considerable adhesion of toner material on the surface of individual carrier particles also occurred.

Furthermore, the use of comparison developer 2 incurred a smaller triboelectricity even in the initial stage of continuous 30000-sheet copying operation, and an obtained image was not sharp, showing minor fog, imaging failure and uneven imaging. In addition, the above problems further deteriorated after the completion of 30000-sheet copying operation, because of further decreased toner triboelectricity. Also, considerable adhesion of toner material on the surface of individual carrier particles also occurred.

The use of comparison developer 3 incurred imaging failure and uneven imaging on an obtained image during the initial stage of continuous 30000-sheet copying operation, and the carrier adhesion on the latent image carrying member was also found. After the completion of 30000-sheet copying operation, the toner triboelectricity further decreased, and accordingly, the obtained image is not sharp, showing minor fog, as well as imaging failure and uneven imageing. Also, considerable carrier adhesion on the latent image carrying member as well as considerable adhesion of toner substance on the surface of individual carrier particles also occurred.

### Test 2 by actual copying operation

A test was performed in a manner identical to the above test 1 by actual copying operation except that the modified developing conditions below were used. The results similar to those of test 1 were obtained.

### [Developing conditions (reverse developing)]

o Latent image carrying member: 140 mm dia. drum type photosensitive member having organic
o photoconductive photosensitive layer
o Linear velocity: 60 mm/sec
o Surface potential: -700 V (image area) to -50 V (non- image area)
o Diameter of developing sleeve: 20 mm
o Linear velocity of developing sleeve: 250 mm/s (forward direction)
o Total number of poles on magnetic roll: 8 poles
o Rotational speed of magnetic roll: 1000 rpm
o Thin layer forming member: 3 mm thick resilient plate made or urethane rubber, being pressed on the surface of developing sleeve
o Development gap: 500 um
o Thickness of developer layer: 400 um (maximum value)
o Toner content in developer: 10 weight%
o Toner content in developer layer formed on developing sleeve: 0.4 mg/cm²
o DC bias voltage: -500 to -600 V
o AC bias voltage: 1.0 to 2.5 kV (frequency, 3 kHz; peak-peak value)

### (Example 2)

Fig. 5 schematically illustrates the constitution of another example of an image forming apparatus used in embodying the developing method, wherein an image input unit IN is unit-built and comprises an illuminating light source 1, a mirror 22, a lens 23 and one-dimensional color CCD image sensor 24. The image input unit IN is shifted in the direction shown by an arrow x with an unshown driving mechanism, and the CCD image sensor 24 reads an original draft. Instead, with the image input unit IN being stationary, a draft table may be shifted to shift the original draft 25.

The image information read by the image input unit IN is converted into data suitable for recording at an image processing unit TR. A laser optical system 26 forms a latent image on the image carrying member 20 in the following manner and based on the above-mentioned image data. The surface of image carrying member 20 is uniformly electrified with a Scorotron electrification electrode 27. Then, image exposure light L with the recorded data incorporate is illuminated from the laser optical system 26 via a lens upon the image forming member 20. In this way, an electrostatic latent image corresponding to the original draft is formed on the latent image carrying member 20.

The electrostatic latent image is developed by a developing unit A containing yellow toner B. The latent image carrying member 20 on which a toner image has been formed is again uniformly electrified by the Scorotron electrification electrode 27 and receives image exposure light L into which recorded data of another color element has been incorporated. The formed electrostatic latent image is developed by a developing unit B containing magenta toner C.

As a result, a two-color toner image of yellow toner B and magenta toner C is formed on the image carrying member 20. Similarly, a cyan toner D image as well as a black toner A image are consecutively superposed on the two-color toner image to form a four-color toner image on the latent image carrying member 20. Additionally, the developing units A, B, C, and D respectively containing each color toner commonly have the constitution similar to that of the developing unit in Fig. 1.

A multicolor toner image obtained in such a manner is transferred on a recording paper P with a transfer electrode 29 after being electrically neutralized for each transfer by an exposure lamp 28. The recording paper P is separated by a separation electrode 30 from the latent image carrying member 20 and is fixed with a fixer 31, thus forming a fixed image. At the same time, the triboelectricity on the image carrying member 20 is neutralized by a neutralization electrode 32, and the surface of which is cleaned by a cleaning mechanism 33.

The cleaning mechanism 33 in this example has a cleaning blade 34 and a fur brush 35 which are kept out of contact with the latent image carrying member 20 during formation of an image. Once a multicolor image is finally formed on the latent image carrying member 20, the cleaning blade 34 and the fur brush 35 come in contact with the latent image carrying member 20 and scrape off toner left untransferred on the member 20. Then, the cleaning blade 34 leaves the latent image carrying member 20, and, a little later, the fur brush also leaves the latent image carrying member. The fur brush 35 functions to remove toner left on the latent image carrying member 20 after the cleaning blade 34 leaves the member 20. Numeral 36 denotes a roller which collects toner scraped off by the blade 34.

A typical example of laser optical system 26 is shown in Fig. 9. In this figure, numeral 37 denotes a semiconductor laser generator, numeral 38 a rotatable polygon mirror, and numeral 39 a fθ lens.

In such an image forming apparatus, it is advantageous to carry out with a timing for starting imagewise exposure by providing an optical reference mark for positioning of each image on the latent image carrying member 20 and by reading the mark by an optical sensor or the like.

### Test 3 by actual copying operation

Using the image forming apparatus, a test operation to form 30000 sheets of copied image was performed so as to examine the triboelectricity on toner, fog, adhesion of carrier on a latent image carrying member, imaging failure, and uneven imaging. The results are listed in Table 2 shown later.

In this test by actual copying operation, a reverse developing method schematically shown in Fig. 6 was performed, whereby the image forming process was performed based on the operation timings (in this figure a higher level corresponds to an ON status) listed in Fig. 7.

Fig. 6 schematically illustrates the change in the surface potential of latent image carrying member having a positive triboelectrical polarity. PH represents an exposure area in the latent image carrying member, DA a non-exposure area in the similar member, and DUP an increase in potential due to the adhesion of positive-charged toner T₁ area PH caused by the first development.

The latent image carrying member is uniformly electrified with a Scorotron electrode, so as to have a specific positive surface potential E as shown in Fig. 6-(1). Next, the first imagewise exposure is effected by an exposure light source such as a laser, cathode ray tube, LED or the like, whereby the potential of exposure area PH drops in proportion to the light amount as shown in Fig. 6-(2). An electrostatic latent image formed in this way is developed by a developing unit to which a positive bias voltage approximately equal to the surface potential E on the non-exposure area is applied. As a result, a positive-charged toner T₁ adheres to the exposure area PH having a relatively low potential as shown in Fig. 6-(3), thus the first toner image is formed. The potential in this areas where the toner image having been formed increases by DUP, since the positive-charged toner T₁ has adhered there. However, the potential still differs from that of the non-exposed area DA. Next, the surface of latent image carrying member where the first toner image has been formed is subjected to the second electrification by the electrifier, as a result, whichever the toner T₁ is present or not, uniform surface potential E is attained, as shown in Fig. 6-(4). The surface of latent image carrying member is further subjected to the second imagewise exposure, which forms an electrostatic latent image, as shown in Fig. 6-(5). The electrostatic latent image is, similarly to the above description, developed with a positive-charged toner T2whose color different from that of the toner T₁. This step forms the second toner image shown in Fig. 6-(6).

With the above toner image forming process being repeated, a multicolor toner image is formed on the latent image carrying member. Then, the multicolor toner image is transferred onto a recording paper, which is heated or pressed to fix the image. Thus, the multicolor recorded image is finally formed. Toner and triboelectrical potential on the surface of latent image carrying member are removed, and the next sequence of multicolor image forming is prepared. Additionally, it is also possible to use a method to fix a multicolor toner image directly onto the latent image carrying member. In the developing method illustrated in Fig. 6, it is favorable that the processing step in Fig. 6-(6) be performed without allowing the developer layer to come in contact with the surface of latent image carrying member.

### [Developing conditions (reverse developing) and others]

o Latent image carrying member: 140 mm dia. drum type photosensitive member having organic photoconductive photosensitive layer
o Linear velocity: 60 mm/sec
o Surface potential: -700 V (non-image area) to -50 V (image area)
o Exposure light source: Semiconductor laser (wavelength, 780 nm; recording density, 16 dots/mm)
o Constitution of developing units A through D
   Diameter of developing sleeve: 20 mm
   Unear velocity of developing sleeve: 250 mm/s (forward direction)
   Total number of poles on magnetic roll: 8 poles
   Rotational speed of magnetic roll: 800 rpm
   Thin layer forming member: 3 mm thick resilient plate made of urethane rubber, being pressed on the surface of developing sleeve
   Development gap: 0.4 mm
   Maximum magnetic flux density on surface of developing sleeve: 700 gauss
   Thickness of developer layer: 250 µm (maximum value)
   Toner content in developer layer formed on sloping sleeve: 0.8 mg/cm²
   DC bias voltage during developing: -500 V
   AC bias voltage during developing: 1.2 kV
   (Frequency, 2 kHz; peak-peak value)
   DC bias voltage during non-developing: 0 V
   AC bias voltage during non-developing: Higher than 0.3 kV
   (Frequency, 2 kHz; peak-peak value)
   (During non-developing, magnetic roll and developing sleeve are stationary. Developing sleeve may be electrically floated.)
o Developing sequence: (Yellow) → (Magenta) → (Cyan) → (Black)
o Transfer process: Corona discharge method
o Fixing process: Heat roll method
o Cleaning process: Blade and fur brush

As can be understood from the results listed in Table 2, when executing the developing method described, the toner demonstrated a proper triboelectricity, and a sharp color image featuring high-resolution as well as excellent gradation reproducibility is formed without accompanying any of fog, carrier adhesion of the image carrying member, imaging failure, and uneven imaging.

The developing method is capable of providing a sharp image, whose quality is comparable to that of the first copied image, even after 30000 sheet-copying operation. Additionally, inspection of the contamination in an image. forming apparatus, confirmed only an extremely limited contamination with toner and carrier.

### (Example 3)

Fig. 8 schematically illustrate the outline of another example of image forming apparatus used for embodying the developing method described. This image forming apparatus has a constitution, wherein a multicolor toner image is formed at once, while a latent image carrying members completes one rotation. The image forming apparatus in Fig. 8 differs from the apparatus in Fig. 5 in that:
(1) Developing units A through D individually have electrification electrodes, respectively, 27A, 27B, 27C and 27D, and laser optical systems, respectively, 26A, 26B, 26C and 26D, in order to enable the developing processes with all the color toners to be sequentially performed, and;
(2) A cleaning mechanism 33 comprises a cleaning blade 34 and a roller 36 for collecting toner, and, the cleaning blade 34 is always being pressed upon the latent image carrying member 20, and;
(3) The appratus has a transporting path, for a recording paper P, which is different from that of the apparatus in Fig. 5.

When forming, for example, a four-color image with this image forming apparatus, and even if the linear velocity of the latent image carrying member is set equal to that of the apparatus in Fig. 5, the image may be formed approximately four times swiftly than with the latter apparatus.

### Test 4 by actual copying operation

Using the image forming apparatus in Fig. 8, and by actually applying the developing method described, a test operation to form 30000 sheets of copied image was performed so as to examine, respectively in the initial stage of image forming operation and after the completion of 30000-sheet copying operation, the triboelectricity on toner, fog, adhesion of carrier on a latent image carrying member, imaging failure, and uneven imaging. The results were as satisfactory as those of the previously mentioned test 3 by actual copying operation.

In this test by actual copying operation, an image forming process in compliance with the following developing conditions was exercised.

### [Developing conditions (reverse developing) and others]

o Latent image carrying member: 140 mm dia. drum type photosensitive member having organic photoconductive photosensitive layer
o Linear velocity: 200 mm/sec
o Surface potential: -700 V (non-image area) to -50 V (image area)
o Exposure light source: Semiconductor laser (wavelength, 780 nm; recording density, 16 dots/mm)
o Constitution of developing units A through D
   Diameter of developing sleeve: 20 mm
   Linear velocity of developing sleeve: 500 mm/s (forward direction)
   Total number of poles on magnetic roll: 8 poles
   Rotational speed of magnetic roll: 1500 rpm
   Thin layer forming member: 3 mm thick resilient plate made of urethane rubber, being pressed on the surface of developing sleeve
   Development gap: 0.3 µm
   Maximum magnetic flux density on surface of developing sleeve: 700 gauss
   Thickness of developer layer: 250 µm (maximum value)
   Toner content in developer layer formed on developing sleeve: 0.6 mg/cm²
   DC bias voltage during developing: -500 V
   AC bias voltage during developing: 2.0 kV (Frequency, 3 kHz; peak-peak value)
   DC bias voltage during non-developing: 0 V
   AC bias voltage during non-developing: More than 0.3 kV
   (Frequency, 2 kHz; peak-peak value)
   (During non-developing, magnetic roll and developing sleeve are stationary. Developing sleeve may be electrically floated.)
o Developing sequence: (Yellow) → (Magenta) → (Cyan) → (Black)
o Transfer process: Corona discharge method
o Fixing process: Heat roll method
o Cleaning process: Blade system

Additionally, in this test 4 by actual operation, the color development sequence may be modified; for example, (black) → (yellow) → (magenta) → (cyan).

### (Example 4)

Next, one example using a resin-coated carrier comprising magnetic particles individually coated with resin containing more than 30 weight% fluoro resin is described below.

Using the image forming apparatus in Fig. 3, a test was performed in a manner identical to that of Example 1, but using the developing method of the present invention.

### Preparation of resin-coated carrier

### (1) Carrier X

26 g vinylidene fluoride-tetrafluoro ethylene copolymer (copolymerization molar ratio, 80:20; intrinsic viscosity, 0.95 dl/g; manufactured by Daikin Kogyo Co., Ltd.) was dissolved in 800 ml acetone-methyethyl ketone (weight ratio, 1:1) mix solution to prepare a coating solution.

Using a Spiller Coater manufactured by Okada Seiko-sha Co., Ltd., the coating solution was applied to copper-zinc ferrite particles (particle size distribution, 15 to 60 um; weight-average particle size, 35 um), whereby heating with 100° C temperature was performed to prepared carrier having individual particles being coated with resin containing fluororesin. The thickness of coating layer was 1.0 µm. This carrier was designated carrier X.

The properties of the carrier X were as follows:

| | |
|---|---|
| Weight-average particle size | 35 µm |
| Magnetization | 20 emu/g (Measured magnetic field: 1000 Oe) |
| Resistivity | More than 10¹⁴ Ω.cm |

### (2) Carrier Y

A carrier having particles individually being coated with a 1.0 um thick fluoro resin layer was prepared in a manner identical to that of carrier X except that a polymer comprising monomer represented by the following general formula was used instead of the vinylidene fluoride-tetrafluoro ethylene copolymer. This carrier was designated carrier Y. (Intrinsic viscosity of polymer = 0.59 dl/g)

The properties of the carrier Y were as follows:

| | |
|---|---|
| Weight-average particle size | 40 µm |
| Magnetization | 20 emu/g (Measured magnetic field: 1000 Oe) |
| Resistivity | More than 10¹⁴ Ω.cm |

### (3) Carrier Z

A carrier having particles individually being coated with a 1.0 um thick fluoro resin layer was prepared in a manner identical to that of carrier X except that blend polymer of the polymers (1) and (2) (weight ratio = 7:3) specified below was used instead of the vinylidene fluoride-tetrafluoro ethylene copolymer. This carrier was designated carrier Z.

Polymer (1): Vinylidene fluoride-tetrafluoro ethylene copolymer (copolymeric molar ratio, 80:200; intrinsic viscosity, 0.95 dℓ/g)

Polymer (2): Methyl methacrylate copolymer, Acrypet MF, manufactured by Mitsubishi Rayon Co., Ltd.

The properties of the carrier Z are as follows:

| | |
|---|---|
| Weight-average particle size | 40 µm |
| Magnetization | 20 emu/g (Measured magnetic field: 1000 Oe) |
| Resistivity | More than 10¹⁴ Ω.cm |

### (4) Comparison carrier x

A carrier comprising copper-zinc ferrite particles identical to those of carrier X was prepared. This was designated comparison carrier x.

The properties of the comparison carrier x were as follows:

| | |
|---|---|
| Weight-average particle size | 38 µm |
| Magnetization | 22 emu/g (Measured magnetic field: 1000 Oe) |
| Resistivity | More than 10¹⁰ Ω.cm |

### (5) Comparison carrier y

A carrier having particles individually have a coating layer of 1.0 µm thick styrene resin was prepared in a manner identical to that of carrier X except that styrene (weight-average molecular weight Mw, 71,000; number-average molecular weight Mn, 32,000; glass transition point Tg, 125° C) was used instead of vinylidene fluoride-tetarfluoro ethylene copolymer. This carrier was designated comparison carrier y.

The properties of the comparison carrier y were as follows:

| | |
|---|---|
| Weight-average particle size | 30 µm |
| Magnetization | 20 emu/g (Measured magnetic field: 1000 Oe) |
| Resistivity | More than 10¹⁴ Ω.cm |

### (6) Comparison carrier z

A carrier having particles individually have a coating layer of 1.0 µm thick styrene resin was prepared in a manner identical to that of carrier X except that methyl methacrylate resin (weight-average molecular weight Mw, 73,000; number-average molecular weight Mn, 33,000; glass transition point Tg, 121° C) was used instead of vinylidene fluoride-tetrafluoro ethylene copolymer. This carrier was designated comparison carrier z.

The properties of the comparison carrier z were as follows:

| | |
|---|---|
| Weight-average particle size | 40 µm |
| Magnetization | 18 emu/g (Measured magnetic field: 1000 Oe) |
| Resistivity | More than 10¹⁴ Ω.cm |

### Preparation of toners

### (1) Black toner O

With a Henschel mixer, 100 parts weight styrene-acryl resin (R-5, manufactured by Sekisui Chemical Co., Ltd.) and 3 parts weight polypropylene (Viscol 660 P, manufactured by Sanyo Kasei Kogyo Co., Ltd.) and 10 parts Carbon Black (Mogal L, manufactured by Cabot) and 2 parts weight positive-type charge controlling agent (P-51, manufactured by Orient Chemicals Co., Ltd.) were mixed, then thoroughly kneaded with a triple-roller at a temperature of 140°C. Further, the mixture, after cooled and crushed, was pulverized with a jet mill and classified to prepare black toner powder having a particle size distribution of 6 to 30 um and a weight-average particle size of 11 µm.

To 100 parts weight of the black toner powder, 0.6 parts weight hydrophobic fine titania particles (T-805, manufactured by Nippon Aerozyl Co., Ltd.) was added, then thoroughly blended by a Henschel mixer to prepare black toner. This toner was designated black toner O. The static bulk density of the black toner O was 0.38 g/cm³.

### (2) Yellow toner P

A yellow toner having a weight-average particle size of 11 um was prepared in a manner identical to that of black toner O except that yellow pigment, Pigment Yellow, was used in the place of Carbon Black. This toner was designated yellow toner P. The static bulk density of the yellow toner P was 0.28 g/cm³.

### (3) Magenta toner Q

A magenta toner having a weight-average particle size of 11 µm was prepared in a manner identical to that of black toner O except that magenta pigment, Permanent Carmine F-5B, was used in the place of Carbon Black. This toner was designated magenta toner Q. The static bulk density of the magenta toner Q was 0.29 g/cm³.

### (4) Cyan toner R

A cyan toner having a weight-average particle size of 11 um was prepared in a manner identical to that of black toner O except that cyan pigment, Pigment Blue 1, was used in the place of Carbon Black This toner was designated cyan toner R. The static bulk density of the cyan toner was 0.27 g/cm³.

### Preparation of developers

The above-mentioned carriers X through Z were indepdendently combined with the black toner O to prepare developers 4 through 6 individually having a toner concentration of 12 weight%. At the same time, the above-mentioned comparison carriers x through z were also combined with the black toner O to correspondingly prepare comparison developer 4 through 6 individually having a toner concentration of 12 weight%.

Additionally, yellow toner P, magenta toner Q and cyan toner R were independently combined with carrier X to correspondingly prepare color developers 4 through 6 individually having a toner concentration of 12 weight%.

### Test 5 by actual copying operation

Using each of these developers, a test was performed by executing copying operation, in accordance with the developing method of the invention based on the below specified developing conditions, for 30,000 sheets, whereby the triboelectricity on toner, fog, adhesion of carrier on a latent image carrying member, imaging failure, and uneven imaging were evaluated on the first and 30000th formed images. The results are listed in Table 3 shown later.

### [Developing conditions (reverse developing)]

o Latent image carrying member: 100 mm dia. drum type photosensitive member made of selenium
o Linear velocity: 100 mm/sec
o Surface potential: + 800 V (non-iamge area) to 0 V (image area)
o Diameter of developing sleeve: 25 mm
   Linear velocity of developing sleeve: 25 mm/s (forward direction)
   Total number of poles on magnetic roll: 8 poles
   Rotational speed of magnetic roll: 1200 rpm
   Thin layer forming member: 3 mm thick resilient plate made of urethane rubber, being pressed on the surface of developing sleeve
   Development gap: 500 µm
   Thickness of developer layer: 400 µm (maximum value)
   Toner content in developer: 12 weight%
   Toner content in developer layer formed on developing sleeve: 0.3 mg/cm²
   DC bias voltage: 600 to 700 V
   AC bias voltage: 0.5 to 2 kV (frequency, 2 kHz; peak-peak value)

The methods of evaluation were identical to those of Example 1.

As can be understood from the results listed in Table 3, when executing the developing method of the invention with any of the developers 4 through 8, the toner demonstrated a proper triboelectricity, and a sharp image featuring high-resolution as well as excellent gradation reproducibility is formed without incurring any of fog, carrier adhesion of the image carrying member, imaging failure, and uneven imaging.

With a fluctuation in toner triboelectricity being small, the developing method of the invention using any of the developers 4 through 6 provides a sharp image, whose quality is comparable to that of the first copied image, even after 30000 sheet-copying operation. Additionally, inspection of the contamination in an image forming apparatus confirmed only an extremely limited contamination with toner and carrier. This is because the fluoro resin to form the coating layer of the carrier used in embodying the invention has a smaller critical surface tension when compared to a resin used to prepare a comparison carrier, and accordingly, the toner substance does not easily adhere to the surface of individual carrier particles. Furthermore, the developing effects of bias voltage was satisfactorily demonstrated.

In contrast, the use of comparison developer 4 incurred a smaller triboelectricity even in the initial stage of continuous 30000-sheet copying operation, and an obtained image was not sharp, showing fog, and uneven imaging. In addition, the above problems further deteriorated after the completion of 30000-sheet copying operation, because of further decreased toner triboelectricity. Also, considerable carrier adhesion on the latent image carrying member, as well as imaging failure were also found.

Furthermore, the use of comparison developer 5 provided a relatively smaller triboelectricity even in the initial stage of continuous 30000-sheet copying operation, and an obtained image was not sharp, showing imaging failure and uneven imaging. In addition, the above problems further deteriorated after the completion of 30000-sheet copying operation, because of further decreased toner triboelectricity. Also, large fog occurred, and minor carrier adhesion on the latent image carrying member was also found.

The use of comparison developer 6 incurred imaging failure and uneven imaging on an obtained image during the initial stage of continuous 30000-sheet copying operation, and the carrier adhesion on the latent image carrying member was also found. After the completion of 30000-sheet copying operation, the toner triboelectricity significantly decreased, and accordingly, the obtained image is not sharp, showing great fog, as well as imaging failure and uneven imaging. Also, minor carrier adhesion on the latent image carrying member also occurred.

### Test 6 by actual copying operation

A test was performed in a manner identical to the above test 5 by actual copying operation'except that the modified developing conditions below were used. The results similar to those of test 5 were attained.

### [Developing conditions (normal developing)]

o Latent image carrying member: 140 mm dia. drum type photosensitive member having organic photoconductive photosensitive layer
o Linear velocity: 60 mm/sec
o Surface potential: -700 V (image area) to -50 V (non-image area)
o Diameter of developing sleeve: 20 mm
o Linear velocity of developing sleeve: 250 mm/s (forward direction)
o Total number of poles on magnetic roll: 8 poles
o Rotational speed of magnetic roll: 1000 rpm
o Thin layer forming member: 0.1 mm thick resilient plate made of phosphor bronze plate being pressed on the surface of developing sleeve
o Development gap: 500 um
o Thickness of developer layer: 400 µm (maximum value)
o Toner content in developer: 12 weight%
o Toner content in developer layer formed on developing sleeve: 0.4 mg/cm²
o DC bias voltage: -100 to -200 V
o AC bias voltage: 0.5 to 2.5 kV (frequency, 2 kHz; peak-peak value)

### (Example 5)

### Test 7 by actual copying operation

Using the image forming apparatus illustrated in Fig. 5 and already described in Example 2, a test operation to form 30000 sheets of copied image was performed, in a manner identical to that of test 3 by actual copying operation, so as to examine, respectively in the initial stage of image forming operation and after the completion of 30000-sheet copying operation, the triboelectricity on toner, fog, adhesion of carrier on a latent image carrying member, imaging failure, and uneven imaging. The results are listed in Table 4 shown later.

In this test by actual copying operation, a reverse developing method schematically shown in Fig. 6 was performed, similarly to the test 3 by actual copying operation, whereby the image forming process was performed based on the operation timings (in Fig. 7 a higher level corresponds to an ON status) listed in Fig. 7.

### [Developing conditions (reverse developing) and others]

o Latent image carrying member: 140 mm dia. drum type photosensitive member having selenium-tellurium photosensitive layer
o Linear velocity: 60 mm/sec
o Surface potential: + 700 V (non-image area) to + 50 V (image area)
o Exposure light source: Semiconductor laser (wavelength, 780 nm; recording density, 16 dots/mm)
o Constitution of developing units A through D
   Diameter of developing sleeve: 20 mm
   Linear velocity of developing sleeve: 250 mm/s (forward direction)
   Total number of poles on magnetic roll: 8 poles
   Rotational speed of magnetic roll: 800 rpm
   Thin layer forming member: 3 mm thick resilient plate made of urethane rubber, being pressed on the surface of developing sleeve
   Development gap: 0.3 mm
   Maximum magnetic flux density on surface of developing sleeve: 700 gauss
   Thickness of developer layer: 250 um (maximum value)
   Toner content in developer layer formed on developing sleeve: 0.3 mg/cm²
   DC bias voltage during developing: + 500 V
   AC bias voltage during developing: 1.2 kV
   (Frequency, 2 kHz; peak-peak value)
   DC bias voltage during non-developing: 0 V
   AC bias voltage during non-developing: More than 0.3 kV
   (Frequency, 2 kHz; peak-peak value)
   (During non-developing, magnetic roll and developing sleeve are stationary. Developing sleeve may be electrically floated.)
o Developing sequence: (yellow) → (Magenta) → (Cyan) → (Black)
o Transfer process: Corona discharge method
o Fixing process: Heat roll method
o Cleaning process: Blade system and fur brush

As can be understood from the results listed in Table 4, when executing the developing method of the invention, the toner demonstrated a proper triboelectricity, and a sharp color image featuring high-resolution as well as excellent gradation reproducibility is formed without accompanying any of fog, carrier adhesion of the image carrying member, imaging failure, and uneven imaging.

The developing method of the invention is capable of providing a sharp image, whose quality is comparable to that of the first copied image, even after 30000 sheet-copying operation. Additionally, inspection of the contamination in an image forming apparatus confirmed only an extremely limited contamination with toner and carrier.

### (Example 6)

### Test 8 by actual copying operation

Using the image forming apparatus illustrated in Fig. 8 and already described in Exmaple 3, a test operation to form 30000 sheets of copied image was performed, in a manner identical to that of test 3 by actual copying operation, so as to examine, respectively in the initial stage of image forming operation and after the completion of 30000-sheet copying operation, the triboelectricity on toner, fog, adhesion of carrier on a latent image carrying member, imaging failure, and uneven imaging. The results were as satisfactory as those of the previously mentioned test 7 by actual copying operation.

In this test by actual copying operation, the image forming process was performed in accordance with the following conditions.

### [Developing conditions (erverse developing) and others]

o Latent image carrying member: 140 mm dia drum type photosensitive member having As₂Se₂ photosensitive layer
o Linear velocity: 200 mm/sec
o Surface potential: + 700 V (non-image area) to + 50 V (image area)
o Exposure light source: Helium-neon laser (wavelength, 632.8 mm; recording density, 16 dots/mm)
o Constitution of developing units A through D
   Diameter of developing sleeve: 20 mm
   Linear velocity of developing sleeve: 50 mm/s (forward direction)
   Total number of poles on magnetic roll: 8 poles
   Rotational speed of magnetic roll: 1500 rpm
   Thin layer forming member: 3 mm thick resilient plate made of urethane rubber, being pressed on the surface of developing sleeve
   Development gap: 500 um
   Maximum magnetic flux density on surface of development sleeve: 700 gauss
   Thickness of developer layer: 400 um (maximum value)
   Toner content in developer layer formed on development sleeve: 0.4 mg/cm²
   DC bias voltage during developing: 600 to 700 V
   AC bias voltage during developing: 0.5 to 2 kV
   (Frequency, 2 kHz; peak-peak value)
   DC bias voltage during non-developing: 0 V
   AC bias voltage during non-developing: More than 0.3 kV
   (Frequency, 2 kHz; peak-peak value)
   (During non-developing, magnetic roll and developing sleeve are stationary. Developing sleeve may be electricallyfloated.)
o Developing sequence: (Yellow) → (Magenta) → (Cyan) → (Black)
o Transfer process: Corona discharge method
o Fixing process: Heat roll method
o Cleaning process: Blade system

Additionally, in this test 8 by actual operation, the color development sequence may be modified; for example, (black) → (yellow) → (magenta) → (cyan).

The typical examples embodying the present invention have been described above. However, the developing method of the invention may be advantageously applied also to an apparatus being capable of forming a multicolor toner image with one imagewise exposure on a latent image carrying member.

With one example of such an apparatus having a latent image carrying member favorably comprising an electroconductive member; photoconductive layer, and insulative layer comprising a plurality of different filters, a multicolor toner image is formed, for example, in the following manner.

By forming an electrical charge on the surface of latent image carrying member, which is then subjected to imagewise exposing, an image patterned on the degrees of interface potential density between an insulative layer and a photoconductive layer, whereby the image is uniformly exposed with a specific color light This procedure forms a pattem representing different potentials on the filter layer on the latent image carrying member, whereby the potential pattern is developed by a developing unit containing a specific color toner in order to form a mono-color toner image.

Next the latent image carrying member is triboelectrically charged to smooth its potential pattern, and subjected to a specific color light different from the above-mentioned specific color light, so as to form a potential pattern on the filter layer of the latent image carrying member, whereby the potential pattern is developed by a developing unit containing a specific color toner different from the above-mentioned specific color. This procedure forms the second color toner iamge as superposed on the first color toner image already formed on the latent image carrying member. Additionally, in performing this type of developing process, at least the second developing onwards should be effected in compliance with non-contact developing method.

Accordingly, the above developing process is repeated for a required number of times to allowing a toner of independent color to adhere onto a corresponding filter layer on the latent image carrying member, and this arrangement can resultingly provide a multicolor image (Refer to Japanese Patent Applications Nos. 83096/1984, 187044/1984, 185440/1984 and 229524/1984, i.e. JP-A-225 855/1985, JP-A-65 262/1986, JP-A-63 856/1986 and JP-A-89 071/1987.

Such a type of multicolor image forming apparatus completes a multicolor image forming with only one sequence of the imagewise exposure, and this in turn precludes the possibility of an image whose independent toner images are not misaligned to each other.

The latent image carrying member may either have a constitution (refer to JP-A-77 857/1986 of Japanese Patent Application No. 199547/1984), wherein a filter is incorporated into the electroconductive substrate side, so as to perform the imagewise exposure as well as uniform exposing on the filter side, or another constitution (refer to Japanese Patent Application No. 201084/1984, i.e. JP-A-77 860/1986).

Additionally, a photosensive layer may either be made of a single layer or have a function-separating constitution comprising both a charge generating layer and a charge transporting layer (refer to Japanese Patent Application No. 245178/1985, i.e. JP-A-105 155 (1987).

Furthermore, a latent image carrying member may have a constitution, wherein the photosensitive layer has color separation function (refer to Japanese Patent Applications Nos. 201085/1984 and 245177/1985, i.e. JP-A-77 861/1986 and JP-A-105 154/1987).

## Claims

1. Non-contact method for developing electrostatic latent images on a latent image carrying member, wherein a developer layer of a two-component type developer is formed on a developer transport member, the two-component type developer comprising toner particles and magnetic carrier particles, and said developer layer having a thickness of not more than 1000 µm is brought to a developer area formed between the latent image carrying member and the developer transport member, the distance between the latent image carrying member and the developer transport member in the developing area is larger than the thickness of said developer layer in the developing area, the developing area being subjected to an oscillatory electric field,
**characterized in that**
the carrier particles are coated with a layer of resin containing fluoro resin in an amount greater than 30 % of the total weight of the resin, the weight-average particle size of the carrier particles is 5 to 50 µm, wherein the fluoro resin comprises at least one polymer of
1) Vinylidene fluoride-tetrafluoroethylene copolymer,
2) polymer comprising a vinyl ether monomer represented by the following formula and having a fluorine atom substituent in the side chain wherein Rf is an alkyl group or aralkyl group having more than one fluorine atom, and
3) polymer comprising a vinyl ketone monomer represented by the following formula and having a fluorine atom substituent in the side chain wherein Rf is an alkyl group or aralkyl group having more than one fluorine atom.

2. The method of claim 1, wherein the thickness of said developer layer is 10 to 500 µm.

3. The method of claim 1, wherein in said developing area a minimum gap between said latent image-carrying member and said developer transport member is 100 to 1000 µm.

4. The method of claim 1, wherein said resin containing fluoro resin contains 40 to 100 % by weight of fluoro resin.

5. The method of claim 1, wherein said resin containing fluoro resin contains 50 to 100 % by weight of fluoro resin.

6. The method of claim 1, wherein the thickness of the resin coating layer is 0.1 to 20 um.

7. The method of claim 1, wherein the the thickness of the resin coating layer is 0.1 to 10 µm.

8. The method of claim 1, wherein the thickness of the resin coating layer is 0.3 to 4 µm.

9. The method of claim 1, wherein the thickness of the resin coating layer is 0.3 to 2 µm.

10. The method of claim 1, wherein said resin coated carrier particles are an insulative carrier having a resistivity of more than 10⁸ Ω^{.}cm.

11. The method of claim 1, wherein said resin coated carrier particles are an insulative carrier having a resistivity of more than 10¹³ Ω^{.}cm.

12. The method of claim 1, wherein said resin coated carrier particles are an insulative carrier having a resistivity of more than 10¹⁴ Ω ^{.} cm.

13. The method of claim 1, wherein said resin coated carrier particles are spherical-shaped particles.

## Patentansprüche

1. Verfahren zum berührungslosen Entwickeln elektrostatischer latenter Bilder auf einem Trägerelement für ein latentes Bild,
- bei dem eine Entwicklerschicht eines Entwicklers vom Zweikomponenten-Typ auf einem Entwickler-Transportelement gebildet wird,
- wobei der Entwickler vom Zweikomponenten-Typ Tonerteilchen und magnetische Trägerteilchen enthält, und die Entwicklerschicht, die eine Dicke von nicht mehr als 1000 µm aufweist, in einen zwischen dem Trägerelement für ein latentes Bild und dem Entwickler-Transportelement ausgebildeten Entwicklungsbereich gebracht wird,
- wobei der Abstand zwischen dem Trägerelement für ein latentes Bild und dem Entwickler-Transportelement im Entwicklungsbereich größer als die Dicke der Entwicklerschicht im Entwicklungsbereich ist,
- wobei der Entwicklungsbereich einem oszillierenden elektrischen Feld ausgesetzt wird,
**dadurch gekennzeichnet,**
- daß die Trägerteilchen mit einer Schicht aus Harz überzogen sind, das Fluoroharz in einer Menge größer als 30% des Gesamtgewichtes des Harzes enthält,
- daß die gewichtsgemittelte Teilchengröße der Trägerteilchen zwischen 5 und 50 µm liegt,
- wobei der Fluoroharz aufweist mindestens einen der Polymere
(1) Vinyliden-Fluorid-Tetrafluoroäthylen-Copolymer,
(2) Polymer mit einem Vinyläthermonomer, dargestellt durch die folgende allgemeine Formel und mit einem Substituenten in der Position eines Fluoratoms in der Seitenkette wobei R_{f} eine Alcylgruppe oder Aralkylgruppe darstellt, die mehr als ein Fluoratom substituiert, und
(3) Polymer mit einem Vinylketonmonomer, dargestellt durch die folgende allgemeine Formel und mit einem Substituenten in der Position eines Fluoratoms in der Seitenkette wobei R_{f} eine Alkylgruppe oder eine Aralcylgruppe darstellt, die mehr als ein Fluoratom substituiert.

2. Verfahren nach Anspruch 1, bei dem die Dicke der Entwicklerschicht 10 bis 500 µm beträgt.

3. Verfahren nach Anspruch 1, bei dem in dem Entwicklungsbereich ein minimaler Spalt zwischen dem Trägerelement für ein latentes Bild und dem Entwicklertransportelement 100 bis 1000 µm beträgt.

4. Verfahren nach Anspruch 1, bei dem das Fluoroharz enthaltende Harz 40 bis 100 Gewichts-% Fluoroharz enthält.

5. Verfahren nach Anspruch 1, bei dem das Fluoroharz enthaltende Harz 50 bis 100 Gewichts-% Fluoroharz enthält.

6. Verfahren nach Anspruch 1, bei dem die Dicke der Harzüberzugsschicht 0.1 bis 20 µm beträgt.

7. Verfahren nach Anspruch 1, bei dem die Dicke der Harzüberzügsschicht 0.1 bis 10 µm beträgt.

8. Verfahren nach Anspruch 1, bei dem die Dicke der Harzüberzugsschicht 0.3 bis 4 µm beträgt.

9. Verfahren nach Anspruch 1, bei dem die Dicke der Harzüberzugsschicht 0.3 bis 2 µm beträgt.

10. Verfahren nach Anspruch 1, bei dem die mit Harz überzogenen Trägerteilchen ein Isolationsträger mit einem spezifischen Widerstand von mehr als 10⁸ Ω.cm sind.

11. Verfahren nach Anspruch 1, bei dem die mit Harz überzogenen Trägerteilchen ein Isolationsträger mit einem spezifischen Widerstand von mehr als 10¹³ Ω.cm sind.

12. Verfahren nach Anspruch 1, bei dem die mit Harz überzogenen Trägerteilchen ein Isolationsträger mit einem spezifischen Widerstand von mehr als 10¹⁴ Ω.cm sind.

13. Verfahren nach Anspruch 1, bei dem die mit Harz überzogenen Trägerteilchen kugelförmige Teilchen sind.

## Revendications

1. Procédé par non contact pour développer des images latentes électrostatiques sur un élément porteur d'image latente, dans lequel une couche de révélateur du type à deux composants est formée sur un élément de transport de révélateur, ledit révélateur du type à deux composants comprenant des particules de toner et des particules de vecteur magnétique, et ladite couche de révélateur possédant une épaisseur ne dépassant pas 1 000 µm, est conduite à une zone de développement formée entre l'élément porteur d'image latente et l'élément de transport de révélateur, la distance est l'élément porteur d'image latente et l'élément de transport de révélateur étant supérieure à l'épaisseur de ladite couche de révélateur dans la zone de développement, la zone de développement étant soumise à un champ électrique oscillant, caractérisé en ce que lesdites particules de vecteur sont revêtues d'une couche de résine contenant une résine fluorée en une proportion supérieure à 30 % du poids total de la résine, la granulométrie moyenne en poids des particules de vecteur est de 5 à 50 micron, dans laquelle la résine fluorée comprend au moins un des polymères suivants :
1) copolymère fluorure de vinylidène-tétrafluoroéthylène,
2) polymère comprenant un monomère éther de vinyle représenté par la formule suivante et ayant à titre de substituant un atome de fluor dans la chaîne latérale dans laquelle R_{f} est un groupement alkyle ou un groupement arylalkyle ayant plus d'un atome de fluor et
3) polymère comprenant un monomère cétonevinylique représenté par la formule suivante et ayant à titre de substituant un atome de fluor dans la chaîne latérale dans laquelle R_{f} est un groupement alkyle ou un groupement arylalkyle ayant plus d'un atome de fluor.

2. Procédé selon la revendication 1, dans lequel l'épaisseur des particules de développeur est 10 à 500 µm.

3. Procédé selon la revendication 1, dans lequel dans ladite zone de développement il y a un entrefer minimum entre ledit élément porteur d'image latente et ledit élément de transport de développeur de 100 à 1000 µm.

4. Procédé selon la revendication 1, dans lequel ladite résine contenant de la fluororésine contient 40 à 100 % en poids de fluororésine.

5. Procédé selon la revendication 1, dans lequel ladite résine contenant de la fluororésine contient 50 à 100 % en poids de fluororésine.

6. Procédé selon la revendication 1, dans lequel l'épaisseur du couche couvert de résine est 0.1 à 20 um.

7. Procédé selon la revendication 1, dans lequel l'épaisseur du couche couvert de résine est 0.1 à 10 µm.

8. Procédé selon la revendication 1, dans lequel l'épaisseur du couche couvert de résine est 0.3 à 4 µm.

9. Procédé selon la revendication 1, dans lequel l'épaisseur du couche couvert de résine est 0.3 à 2 µm.

10. Procédé selon la revendication 1, dans lequel lesdites particules porteur couvertes de résine sont un porteur isolant ayant une résistance spécifique de plus de 10⁸ Ω·cm.

11. Procédé selon la revendication 1, dans lequel lesdites particules porteur couvertes de résine sont un porteur isolant ayant une résistance spécifique de plus de 10¹³ Ω·cm.

12. Procédé selon la revendication 1, dans lequel lesdites particules porteur couvertes de résine sont un porteur isolant ayant une résistance spécifique de plus de 10¹⁴ Ω·cm.

13. Procédé selon la revendication 1, dans lequel lesdites particules porteur couvertes de résine sont des particules de forme sphérique.
